

Oct. 5, 1937.

G. WILMANNS ET AL

2,095,018

MANUFACTURE OF ANTIHALATION LAYERS

Filed Oct. 1, 1934

*Fig. 1*



light sensitive emulsion  
layer

support

anti-halation layer of  
gelatine containing  
pyrolusite particles of  
.1 to 5u in diameter

*Fig. 2*



light sensitive emulsion  
layer

anti-halation layer of  
gelatine containing  
pyrolusite particles of  
.1 to 5u in diameter

support

*Fig. 3*



anti-halation layer of  
gelatine containing  
pyrolusite particles of  
.1 to 5u in diameter

light sensitive emulsion  
layer

support

INVENTORS:

Gustav Wilmanns,  
Wilhelm Schneider,  
By Potter, Pearce & Schaffler,

ATTORNEYS.

## UNITED STATES PATENT OFFICE

2,095,018

## MANUFACTURE OF ANTIHALATION LAYERS

Gustav Wilmanns, Wolfen kreis Bitterfeld, and  
Wilhelm Schneider, Dessau in Anhalt, Germany, assignors to Agfa Ansco Corporation, Binghamton, N. Y., a corporation of New York

Application October 1, 1934, Serial No. 746,474  
In Germany October 4, 1933

3 Claims. (Cl. 95—8)

Our present invention relates to the manufacture of anti-halation layers and more particularly to the manufacture of anti-halation layers from pyrolusite.

5 One of its objects is a process for the manufacture of improved anti-halation layers from pyrolusite. Another object is the improved anti-halation layers. Further objects will be seen from the detailed specification following here-  
10 after.

It is known practice to use so-called pyrolusite layers, consisting of higher hydrated oxides of manganese in gelatin, as anti-halation layers. This pyrolusite is produced in the gelatin in col-  
15 loidal form by causing potassium permanganate solution to act on gelatin or by reducing potas-  
sium permanganate by means of manganese salts in the presence of gelatin or other colloid to form manganese dioxide. In neither case,  
20 however, is the pyrosulite present in the form of pure manganese dioxide, but in the form of a mixture of strongly reactive hydrates of varying composition. The anti-halation layers and filter layers containing such a reactive pyrolusite, af-  
25 fect adversely the photographic emulsion when they come into contact therewith.

According to this invention a photographically satisfactory anti-halation layer and filter layer is obtained on the one hand by bringing the size 30 of the particles of pyrolusite to about 0.1 to 5 $\mu$ , and on the other hand by thermally treating, for example, by an intense drying at about 100° C. to 160° C. the pyrolusite, so that no higher hydrates are present. Thus, for example, a suitable pyrolusite can be produced by reduction of potas-  
35 sium permanganate (with alcohol, for example) in aqueous solution. After the pyrolusite formed has been separated it is dried at about 130° C. It  
40 may then, if necessary, be ground in known manner; and when a suspension of it in a colloid swellable in water such as gelatin or casein is cast as an anti-halation layer, the layer exhibits none of the harmful effects on the photographic  
45 emulsion which are caused by colloidal pyrolusite in the gelatin.

The pyrolusite of the anti-halation filter layers according to this invention is soluble in the fixing

bath so that the layers are decolorized in this bath.

The following examples when taken with the accompanying self-explanatory drawing illus-  
5 trate the invention:

32 grams of pyrolusite which have been pre-  
pared as above described and dried at 130° C. and have a grain size between 0.2 and 4 $\mu$  are suspended in a solution of 70 grams of gelatin in 1000 cc. of water. This solution is cast on 10 the back of a photographic film as in Figure 1 or as an intermediate layer between the light sen-  
sitive emulsion layer and the support to form an anti-halation layer as in Figure 2, or on the emulsion layer to form a filter layer as in Fig-  
15 ure 3.

What we claim is:

1. A process of manufacturing anti-halation layers or filter layers which comprises producing pyrolusite from potassium permanganate by re-  
duction, drying said pyrolusite at a temperature 20 between about 100° C. and 160° C., disintegrating the dried pyrolusite to particles of about 0.1 to 5 $\mu$  diameter, suspending said disintegrated pyro-  
lusite in the solution of a colloid swellable in wa-  
ter, and casting said suspension to form an anti-  
halation layer or filter layer.

2. A process of manufacturing anti-halation layers or filter layers which comprises producing pyrolusite from potassium permanganate by re-  
duction, drying said pyrolusite at a temperature 30 of about 130° C., disintegrating the dried pyro-  
lusite to particles of about 0.1 to 5 $\mu$  diameter, sus-  
pensing said disintegrated pyrolusite in the solu-  
tion of a colloid swellable in water, and casting 35 said suspension to form an anti-halation layer or filter layer.

3. A process of manufacturing anti-halation layers or filter layers which comprises producing pyrolusite from potassium permanganate by re-  
duction, drying said pyrolusite at a temperature 40 of about 130° C., disintegrating the dried pyro-  
lusite to particles of about 0.1 to 5 $\mu$  diameter, sus-  
pensing said disintegrated pyrolusite in a so-  
lution of gelatin, and casting said suspension to 45 form an anti-halation layer or filter layer.

GUSTAV WILMANNS.  
WILHELM SCHNEIDER.